

## UNITED STATES PATENT OFFICE

2,269,481

## PRODUCTION OF COLORED PHOTOGRAPHIC IMAGES

John Hubert Reindorp, Ilford, England, assignor to Ilford Limited, Ilford, Essex, England, a British company

No Drawing. Application July 24, 1939, Serial No. 286,281. In Great Britain August 3, 1938

13 Claims. (Cl. 95—6)

This invention relates to the production of colored photographic images by color development.

It is known that a colored image may be formed simultaneously with the silver image obtained by developing a silver halide emulsion with an aromatic amino developing agent if a substance known as a color former is present, for example, in the developing solution or in the silver halide emulsion. The colored image may be revealed by bleaching out the silver image with Farmer's Reducer or other photographic bleaching agent.

It is an object of this invention to provide a new range of color formers. A further object of the invention is to provide a method of producing color photographic images with the aid of such color formers and a still further object is to provide light sensitive silver halide photographic materials containing the new color formers.

Other objects of the invention will appear hereinafter.

According to the present invention in a process of color development in which a silver halide photographic emulsion is developed with an aromatic amino compound as a developer in the presence of a color-former, the color-former employed is a malonic acid mono-ester mono-amide i. e. an organic compound of the general formula:



where  $R_1$  and  $R_2$  represent hydrogen atoms or alkyl, aryl, aralkyl or heterocyclic groups (although they do not necessarily represent the same atoms or groups) or they represent groups linked together as a single cyclic grouping, and  $R_3$  represents an alkyl, aryl or aralkyl group. Thus, for example,  $R_1$  may be a hydrogen atom, a methyl, ethyl, propyl or other alkyl group, a phenyl or other aryl group, a benzyl or other aralkyl group, a thiazole, thiazoline, oxazole, oxazoline, selenazole, selenazoline, pyridine, quinoline, indolenine, diazine (e. g. pyrimidine, and quinazoline) thiodiazole group, or a substituted or unsubstituted polycyclic group such as the benzthiazole, naphthothiazole and anthrathiazole groups.  $R_2$  may also be a hydrogen atom or any of the above mentioned groups although in any one compound it is not necessarily the same as  $R_1$ . Further,  $R_1$  and  $R_2$  may together form a single cyclic grouping, for example, a

pyridine, quinoline, piperidine, pyrazole or indolegroup.  $R_3$  may be, for example, a methyl ethyl, propyl or butyl group, a phenyl group or a benzyl group.

5 The groups  $R_1$ ,  $R_2$  and  $R_3$  may themselves be substituted, e. g. by halogen atoms, by alkyl, aryl, aralkyl and other hydrocarbon groups, or by nitro groups, hydroxy groups, amino groups, substituted amino groups, alkoxy groups or carbethoxy-alkyl groups. Those compounds which contain substituted alkoxy groups yield, in general, colors of especial brilliance.

The preferred compounds for use according to the present invention are compounds of the type described above where  $R_1$  is a hydrogen atom and  $R_2$  is a substituted or unsubstituted phenyl group, suitable substituents in the phenyl group being halogen atoms or nitro, hydroxy, alkoxy or amino groups. Typical compounds of this type are malonis acid mono ethyl ester mono-o-anisidine and malonic acid mono ethyl ester mono-o-chloranilide.

The compounds to be used as color formers in accordance with the invention may be prepared by any suitable method. A convenient method is to condense a compound of the type  $X-CO-CH_2-COOR_3$  where  $R_3$  has the meaning assigned to it above and  $X$  is a halogen atom or an alkoxy group with a compound of the type



35 where  $R_1$  and  $R_2$  have the meanings assigned to them above. Thus, for example, malonic acid mono ethyl ester mono-o-anisidine may be prepared by condensing malonic acid monoethyl-ester mono acid chloride or malonic acid diethyl ester with o-anisidine. Malonic acid mono 40 ethyl ester mono-o-chloranilide may be prepared by a similar condensation using o-chloraniline instead of o-anisidine.

The color-formers of the invention may be incorporated in the developing solution or in the photographic silver halide emulsion. In general, they are very insoluble in water and have little tendency to diffuse from one layer to another when incorporated in the emulsion layers of a multi-layer film or to diffuse into processing 50 baths. Moreover, the compounds show a good resistance to the bleaching action of the sulphites frequently included in developing compositions.

Suitable aromatic amino compounds which may be employed as the developers in conjunction with the color-formers of this invention are

derivatives of p-phenylene diamines and particularly of the asymmetric dialkyl-p-phenylene diamines, e. g. p-aminodimethylaniline, p-aminodiethylaniline and p-aminodibutylaniline. Other developing agents which may be used include p-phenylene-diamine itself, p-methylaminoaniline, p-ethylaminoaniline and p-aminophenol, N,N-diethyl-o-phenylene-diamine, chloro-p-phenylene-diamine, 1,2,5-toluylenediamine, 2-amino-5-diethylaminotoluene, N-p-aminophenylpiperidine, N-methyl-N-hydroxyethyl-p-phenylenediamine, N-butyl-N-hydroxyethyl-p-phenylenediamine, 2-amino-5-(N-β-hydroxyethyl-N-butyl) aminotoluene and its dihydrochloride and α-γ-dihydroxypropyl-p-phenylene diamine. These aromatic amino-developing agents may be used in the form of their salts, which may be either inorganic or organic. The salts are in general more stable than the free bases. As examples of suitable salts mention is made of the hydrochlorides, sulfates and acetates.

In the succeeding examples, the following solution is given by way of example as illustrating the nature of developing solutions which may be employed embodying a color former in accordance with the invention.

*Developing solution A*

|                                                                       |       |      |
|-----------------------------------------------------------------------|-------|------|
| Diethyl-p-phenylenediaminehydrochloride                               | grams | 1    |
| Sodium carbonate (crystals)                                           |       |      |
| Na <sub>2</sub> CO <sub>3</sub> ·10H <sub>2</sub> O                   | grams | 30   |
| Sodium sulphite (crystals)                                            |       |      |
| Na <sub>2</sub> SO <sub>3</sub> ·7H <sub>2</sub> O                    | grams | 12.5 |
| Color former solution (1% or saturated solution, whichever is weaker) | ccs   | 100  |
| Water to make                                                         | litre | 1    |

The color former is dissolved in a suitable water-miscible solvent such as ethyl alcohol or ethylene glycol mono-methyl ether. The sodium sulphite may be omitted if desired.

A suitable development time, using this solution, is two minutes, at a temperature of 65° F.

The following specific examples illustrate the method of production of the new color formers, and their use:

*EXAMPLE 1*

*Malonic acid mono ethyl ester mono-o-anisidide*



320 gms. of diethylmalonate were dissolved in 400 ccs. of dry xylene, to which a few drops of pyridine were added. The mixture was transferred to a distilling flask and brought to the boil. 100 gms. of o-anisidine dissolved in xylene were then added from a dropping funnel over a period of fifteen minutes. The excess diethylmalonate and xylene were then distilled off under vacuum and the residual solution allowed to cool. The cooled solution was filtered.

The filtrate was then diluted to four times its volume with petroleum ether and cooled in a freezing mixture, whereupon the malonic acid mono ethyl ester mono-o-anisidide separated out. M. P. 63-65° C.

Developing solution A, when including this compound and used for the development of photographic silver halide images, produces a brilliant yellow image together with the silver image.

70

65

55

40

35

30

25

20

15

10

5

**EXAMPLE 2**

*Malonic acid mono ethyl ester mono-β-naphthalide*



This compound was produced by the general method described in Example 1 using 2.00 gms. of diethyl malonate dissolved in 10 ccs. xylene and 1.43 gms. of β-naphthylamine dissolved in 20 ccs. xylene. The product has a melting point of 81° C.

Developing solution A, when including this compound and used for the development of photographic silver halide images, produces a yellow image together with the silver image.

**EXAMPLE 3**

*Malonic acid mono ethyl ester mono-m-nitranilide*



10 ccs. of diethylmalonate and 4.08 gms. of m-nitraniline were heated together in an oil bath for three hours at 130-140° C.

The excess diethylmalonate was then distilled off in vacuo and the residue was warmed with 60 ccs. of dry ethyl alcohol. The mixture was then cooled in a freezing mixture and filtered. The filtrate was evaporated on a water bath to remove the ethyl alcohol and water was added. The mixture was then cooled in ice and filtered. The residue was then boiled up with benzene and filtered hot; the filtrate was evaporated to 10 ccs. and allowed to cool, whereupon yellow crystals of malonic acid mono ethyl ester mono-m-nitranilide separated. M. P. 48° C.

Developing solution A when including this compound and used for the development of photographic silver halide images produces a bright yellow image together with the silver image.

**EXAMPLE 4**

*Malonic acid mono ethyl ester mono-o-hydroxyanilide*



5.45 gms. of o-amino-phenol and 40 gms. of diethylmalonate were heated in an oil bath, for three hours, at 120° C. On cooling, a brown solid, M. P. 106° C. separated and this was recrystallised from benzene. Developing solution A, when including this compound and used for the development of photographic silver halide images produces a deep green image together with the silver image.

**EXAMPLE 5**

*1-ω-carbethoxyacetyl amino benzthiazole*



4.5 gms. of 1-amino-benzthiazole were dissolved by warming in 200 ccs. of xylene and the solution was slowly added to a solution of 9.6 gms. of diethylmalonate in 15 ccs. of xylene and contain-

ing two drops of pyridine, the addition of the 1-amino-benzthiazole being effected over a period of about thirty minutes.

During this process the solutions were maintained at boiling and about 100 ccs. of the xylene was removed. On cooling the products, a yellow solid separated, which on recrystallisation from ethyl alcohol had a melting point of 180° C. Developing solution A when including this compound and used for the development of photographic silver halide images produces an orange-brown image together with the silver image.

#### EXAMPLE 6

This example illustrates the incorporation of the color-formers of this invention in emulsion layers. 20 ccs. of 1% solution in ethylene glycol mono-methyl ether of malonic acid mono-ethyl ester mono-o-anisidide were added to 25 ccs. of 10% aqueous solution of gelatin and the mixture added to 50 ccs. of a melted photographic "Gas-light" emulsion containing approximately 20 gms. of silver halide, principally silver chloride, per pound weight of emulsion. The emulsion thus prepared was coated on a paper support and dried. The emulsion coated paper was exposed under a negative and was then developed with a developing solution of the constitution of Developing solution A excluding the color former but including an equivalent quantity of the water miscible liquid such as ethyl alcohol or ethylene glycol mono methyl ether. A brilliant yellow image was produced together with the silver image.

In each of the above examples the dye image may be revealed by bleaching out the silver image with Farmer's Reducer or other known photographic bleaching agent.

In addition to the specific color formers described above, the following are examples of color formers which may be prepared and used according to this invention:

Malonic acid mono ethyl ester mono-p-anisidide  
 Malonic acid mono ethyl ester mono-p-nitro-anilide  
 Malonic acid mono ethyl ester mono- $\alpha$ - naphthalide  
 1- $\omega$ -carbethoxy acetyl amino-5 - ethoxy - benzthiazole  
 Malonic acid mono ethyl ester mono anilide  
 Malonic acid mono ethyl ester mono-o-nitro-anilide  
 Malonic acid mono ethyl ester mono-p-carbethoxy-anilide  
 N,N'-di-carbethoxyacetyl benzidine  
 1- $\omega$ -carbethoxyacetyl amino-2-hydroxy - 4:5 - di-methylbenzene  
 Malonic acid di-o-hydroxy-p-nitroanilide  
 Malonic acid mono ethyl ester mono-o-chloranilide

The process of development employing the color formers in accordance with the present invention may be applied either to a latent image in an emulsion of a silver halide which has been exposed to the action of light, for example, in a camera or behind a photographic negative image; or it may be applied to the residual silver halide left when an initial reduced silver image has been dissolved away as in the reversal process of development; or it may be applied to a developed photographic image in metallic silver which has been fixed by the removal of unchanged silver halide, and subsequently converted to a developable silver salt by means of known

photographic bleaching agents. In the last two cases the residual silver halide and the silver salt respectively may be made developable by the action of light or in any other way, e. g. by treatment with sodium arsenite.

The production of colored images by means of the color formers of this invention may be applied to colloid layers sensitised by bichromate. Thus the color formers may be incorporated in colloid layers (e. g. gelatin, gum arabic or albumin), the layers exposed, the unexposed colloid removed, e. g. by treatment with hot water, and the color developed in the exposed portions by treatment with p-nitroso-dialkyl-aniline or its derivatives.

I claim:

1. A photographic color forming developer which comprises an aromatic amino developing compound and a color former which is a malonic acid mono-ester mono-amide having a methylene radical attached directly to the two carbonyl radicals of the malonic acid nucleus.

2. A photographic color forming developer which comprises an aromatic amino developing compound and a color former of the general formula:



wherein R<sub>1</sub> and R<sub>2</sub> are groups selected from the class consisting of hydrogen atoms and substituted and unsubstituted hydrocarbon groups and heterocyclic groups, and R<sub>3</sub> is a group selected from the class consisting of substituted and unsubstituted hydrocarbon groups.

3. A photographic color forming developer which comprises an asymmetric di-alkyl-p-phenylene diamine and a color former which is a malonic acid mono-ester mono-amide having a methylene radical attached directly to the two carbonyl radicals of the malonic acid nucleus.

4. A method of producing a colored image in a silver halide emulsion which comprises developing the emulsion with an aromatic amino developing agent in the presence of a color former which is a malonic acid mono-ester mono-amide having a methylene radical attached directly to the two carbonyl radicals of the malonic acid nucleus.

5. A method of producing a colored image in a silver halide emulsion which comprises developing the emulsion with an aromatic amino developing agent in the presence of a color former of the general formula:



wherein R<sub>1</sub> and R<sub>2</sub> are groups selected from the class consisting of hydrogen atoms and substituted and unsubstituted hydrocarbon groups and heterocyclic groups, and R<sub>3</sub> is a group selected from the class consisting of substituted and unsubstituted hydrocarbon groups.

6. A method of producing a colored image in a silver halide emulsion which comprises developing the emulsion with an asymmetrical di-alkyl-p-phenylene diamine in the presence of a color former which is a malonic acid mono-ester mono-amide having a methylene radical attached directly to the two carbonyl radicals of the malonic acid nucleus.

7. A method of producing a colored image in a silver halide emulsion which comprises devel-

oping the emulsion with a developing solution which contains an aromatic amino developing agent and a malonic acid mono-ester mono-amide having a methylene radical attached directly to the two carbonyl radicals of the malonic acid nucleus.

8. A light sensitive silver halide photographic emulsion containing a color former which is a malonic acid mono-ester mono-amide having a methylene radical attached directly to the two carbonyl radicals of the malonic acid nucleus.

9. A photographic element bearing at least one light sensitive silver halide emulsion layer containing a color former of the general formula:



wherein  $R_1$  and  $R_2$  are groups selected from the class consisting of hydrogen atoms and substituted and unsubstituted hydrocarbon groups and heterocyclic groups, and  $R_3$  is a group selected

from the class consisting of substituted and unsubstituted hydrocarbon groups.

10. A light sensitive silver halide emulsion containing as a color former a compound of the general formula:



wherein  $R'$  is an aromatic hydrocarbon radical containing an alkoxy group, and  $R''$  is a lower alkyl group.

11. A light sensitive silver halide emulsion containing as a color former the mono-o-anisidine of malonic acid ethyl ester.

12. A photographic color forming developer comprising an aromatic amino developing compound and the mono-o-anisidine of malonic acid ethyl ester.

13. The process which comprises developing a photographic element bearing silver halide image in the presence of the mono-o-anisidine of malonic acid ethyl ester with a color coupling aromatic amino developing agent containing an unsubstituted amino group.

JOHN HUBERT REINDORP.

CERTIFICATE OF CORRECTION.

Patent No. 2,269,481.

January 13, 1942.

JOHN HUBERT REINDORP.

It is hereby certified that error appears in the printed specification of the above numbered patent requiring correction as follows: Page 1, second column, line 20, for "malonis" read --malonic--; page 2, second column, line 5, in the formula, for "NC" read --NH--; and that the said Letters Patent should be read with this correction therein that the same may conform to the record of the case in the Patent Office.

Signed and sealed this 3rd day of March, A. D. 1942.

(Seal)

Henry Van Arsdale,  
Acting Commissioner of Patents.